

April 2, 1940.

F. HANFF ET AL

2,195,591

TEXTILE FABRIC CONSISTING OF A PLURALITY OF INTERWOVEN LAYERS

Filed June 4, 1937

Fig.1



Fig. 2



Fig. 3



Fig. 4



INVENTOR  
FRITZ HANFF  
BY  
Julius Reimann.  
Fritz Hanff  
ATTORNEY

## UNITED STATES PATENT OFFICE

2,195,591

## TEXTILE FABRIC CONSISTING OF A PLURALITY OF INTERWOVEN LAYERS

Fritz Hanff, Berlin-Wilmersdorf, and Julius Reimann, Wuppertal-Elberfeld, Germany, assignors, by mesne assignments, to Trubenizing Process Corporation, New York, N. Y., a corporation of New York

Application June 4, 1937, Serial No. 146,354  
In Germany June 9, 1936

3 Claims. (Cl. 139—414)

This invention relates to an improved textile fabric consisting of a plurality of interwoven layers forming a so-called multiple weave fabric. The improved textile fabric is mainly intended for the manufacture of wearing apparel, and particularly semi-stiff collars.

For the manufacture of semi-stiff wearing apparel it has heretofore been proposed to employ a multiple weave fabric, comprising a plurality of fabric layers interwoven during the process of weaving. The elasticity and stiffness of articles made of such multiple weave fabric often deteriorate, particularly after prolonged use, and accordingly they are generally treated with starch or other stiffening agents.

It has furthermore been proposed to provide composite fabrics for the manufacture of semi-stiff articles of wearing apparel which composite fabrics consist of a plurality of plies of fabric, one or more of which contain cellulose derivatives or similar binding substances, and wherein the stiffening is obtained, not by interweaving the layers, but by subjecting them to the action of an organic solvent and subsequent pressure with heat to unite the layers and evaporate the solvent.

The present invention relates to the first mentioned type of fabrics, namely multiple weave fabrics, wherein either a warp or several weft layers or several warps and several weft layers are interwoven during the weaving process in known manner.

In the textile fabric according to the invention, consisting of a plurality of interwoven layers (multiple weave fabric) certain of the threads disposed within the fabric and not appearing on the surface consists of binding substances soluble in organic solvent, or contains such substances.

The threads consisting of binding substances may be woven into the layers of fabric as warp threads or as weft threads, or also as part of the warp or weft threads.

In order to give to the improved textile fabric a permanently elastic stiffness, it is treated with a solvent for the said binding substance and is then subjected to the action of heat and pressure.

A textile fabric thus treated has greater elasticity than the multiple weave fabric mentioned above, since owing to the dissolution of the threads of binding substance and their subsequent re-hardening, in conjunction with the resulting adhesive connection with the adjacent threads of the fabric, it is stiffened from inside

permanently and its stiffness is not lost by washing. Wearing apparel made of this fabric does not lose this stiffness even after long wear and repeated washing and therefore does not require to be treated with starch or other stiffening agents.

The improved textile fabric may be used with advantage for the manufacture of articles permeable to air and moisture, particularly semi-stiff collars. It is advisable to maintain the spacing of the threads of the binding substance at such value and to employ them in such numbers that after treatment with the solvent interstices of such size are left that free passage of air and moisture is ensured. It has been found, for example, that a fabric, one-third of the warp threads of which consist of binding substance, will allow air and moisture to pass through very satisfactorily. The quantity of the binding substance employed does not depend solely upon the number of the threads consisting of binding substance, but also upon the thickness of the individual threads.

For example, a textile fabric which will allow the free passage of air and moisture is obtained if in the manufacture 60 threads of 60/2 cotton and 30 cellulose acetate threads of 200 denier are employed per cm. in the direction of the warp and 44 threads of 16/1 cotton per cm. in the direction of the weft.

It has already been proposed to weave threads of cellulose derivative into a simple fabric consisting of one warp and one weft only and to treat the finished fabric with solvents. Apart from the fact that the object of this was to produce a waterproof fabric, in these fabrics the threads of cellulose derivative were exposed on the outer sides of the fabric, so that after the treatment with the solvent the threads to be dissolved smothered the whole surface. Such a fabric was therefore unsuitable for the manufacture of wearing apparel.

As binding substances for the improved textile fabric such substances may be employed, which may be rendered temporarily adhesive by means of organic solvents or swelling agents, such as acetone, methyl alcohol, butyl acetate, dibutyl tartrate, diethyl phthalate and the like, inasmuch as they are dissolved to a greater or lesser extent or are caused to swell by said solvents. Upon treatment of the textile fabric with heat and pressure, whereby the solvent is caused to evaporate, the binding substances lose their adhesiveness and the individual threads of the fabric become stuck together so fast that the

finished textile fabric has increased elasticity resistant to washing as compared to the known multiple weave fabrics for semi-stiff collars and to the fabrics to be treated with starch.

- 5 As binding substances for example cellulose derivatives, such as cellulose acetate and nitro cellulose, artificial resins of low polymerization, as for example resoles made on a phenole base, vinyl artificial resins and the like are suitable.
- 10 These binding substances or the threads made thereof possess to a great extent the properties of natural textile fibres, i. e., they are washable and ironable, elastic and so forth. It has been found that cellulose derivatives, such as for example cellulose acetate, are particularly suitable for the manufacture of the textile material according to the invention. Wearing apparel or parts thereof made of the new textile fabric may be washed in the usual way and after ironing they are again stiff, without treatment with starch being necessary.

The improved textile fabric may be manufactured in various ways. For example, it is possible to provide a fabric having a warp layer 25 and two weft layers with additional warp and weft threads consisting of or containing the aforesaid binding substances. Again, a fabric having a plurality of warp and weft layers, i. e., consisting of two or more interwoven layers of 30 fabric, may be provided with additional warp and weft threads consisting of or containing binding substances. The important point is that the layers of fabric disposed on the outer side do not contain binding substance in the 35 warp or weft. The binding substances must be so disposed between the upper and lower sides of the fabric that they shall not appear on the surface after dissolution and shall not become visible. After solidification a stiff, porous layer 40 is formed between the interwoven layers of fabric and this gives to the whole fabric a permanent stiffness, whereby wearing apparel, for example collars, manufactured thereof permanently 45 retain their shape, without starch or other stiffening agents being applied thereto.

Weft or warp threads which do not consist wholly of binding substances, but merely contain them, may be made for example of a material 50 free of binding substance, such as cotton, artificially spun fibres, artificial silk and the like and wound with threads consisting of the binding substances in question. The threads of material free of binding substances may also be 55 impregnated with the binding substance, for example by using a solution of the binding substance. If artificial silk is used, it must be of a kind which is not soluble in organic solvents, as is for example acetate silk.

Furthermore, it has been found that the improved textile material is particularly suitable for the manufacture of white wearing apparel. It is very comfortable to wear and even when perspiration penetrates it it does not become 65 soft and unsightly.

The invention will be more particularly described with reference to the accompanying drawing, and it is to be particularly understood that these illustrate embodiments merely 70 by way of example and explanation.

Figure 1 is a diagrammatic sectional view of a textile fabric, wherein threads of binding substance are woven into the fabric as warp threads.

Figure 2 is a cross section of a fabric, where- 75 in the threads of binding agent form weft threads.

Figure 3 is a diagrammatic cross section of a collar made of the improved textile fabric.

Figure 4 is a similar view of an alternative construction of collar.

In Figure 1 the threads forming the basic 5 warps of the fabric are indicated at 1 and these are interwoven with the weft threads 2 in such a manner that two weft layers are formed, one above the other. The threads 3, consisting of a binding substance, for example cellulose acetate, form an intermediate layer in the form of additional warps, which are completely concealed by the two weft layers.

In Figure 2 the threads forming the warp are again indicated at 1 and the weft threads of the 15 two normal weft layers are indicated at 2. The weft threads 4, consisting of binding substance, are located between the two weft layers of the fabric and are concealed thereby.

When the binding substance threads shown 20 in Figures 1 and 2 are moistened with a solvent, they become adhesive and when heat and pressure is applied a permanent stiffening of the individual weft and warp layers is effected, whereby an elastic, stiffened fabric is formed. The 25 action of the solvent upon the threads of binding agent is generally so calculated that only partial dissolution thereof, sufficient for stiffening, takes place. However, in some cases it may be desirable to effect complete dissolution of 30 the threads.

In Figures 1 and 2 a fabric of comparatively simple structure is shown. If desired fabrics consisting of several layers of warps and wefts may also be stiffened by the employment of weft or 35 warp threads of binding substances and treatment with organic solvents.

Figure 3 shows an embodiment by way of example of a collar made of the improved textile fabric and comprising two parts. The upper 40 or collar top part 5 and the lower or collar band part 6 of the collar are cut in known manner of the improved fabric and the two parts are interconnected along the seams 7. Around the edge 8 a narrow strip 9 is placed and sewn 45 together with the parts. The collar top 5 and the collar band 6 are hemmed as usual and the free edges 10 and 11 are edged with narrow strips 12 and 13 respectively. When the collar is completed it is moistened with solvent and 50 then stiffening is effected with the aid of a hot press.

While in Figure 3 the manufacture of a two part collar of the improved textile fabric has been explained in detail, it is to be understood 55 that the multiple weave fabric according to the invention is also suitable for the manufacture of one piece collars. In this case it is preferable to omit a few acetate threads during the weaving operation in the zone where the collar is to be 60 folded and to substitute them, if desired, by cotton threads. After treatment with the solvent upon the completion of the collar and the subsequent heat and pressure treatment no stiffening of the fabric occurs along the folding zone, 65 so that the collar may be easily folded therealong and will have a good shape.

An alternative method of making a collar from the new multiple weave material is shown in Figure 4. In this construction only the upper or 70 collar top part 5 of the collar consists of the new multiple weave material. As in the collar of Figure 3, the free edge of the upper or collar top part is bound with a narrow strip 12 secured by a seam 7. The lower or band part 6a of the 75

collar differs from the band 6 collar shown in Figure 3 in that it does not consist of a multiple weave material but is made of three plies of fabric. The two outer plies 14 and 15 consist of ordinary textile fabric while the lining ply 16 consists of woven fabric composed of or containing cellulose acetate threads. The collar top and the band of the collar are connected by a seam 7. The lower edge of the collar top needs no binding and it is sufficient to secure it with a seam 7'. The width of the lining ply 16 is equal only to the finished width of the collar top, whereas in cutting out the outer plies 14 and 15, allowance must be made for the turned in edges.

10 The use of the improved textile fabric is not restricted to collars, it is eminently suitable for the manufacture of a great variety of articles of wearing apparel or parts thereof, such as cuffs, brims, turn ups, shirt fronts, particularly piqué fronts for dress shirts, bathing suits, trimmings of ladies' wear and so forth.

15 What we claim is:

1. A woven textile fabric consisting of a two-weft plane fabric in which the wefts of each plane are separated from those of the other by a stuffer threads lying in an intermediate plane, said stuffer threads comprising an organically

soluble adhesive substance, the warp threads of which fabric pass from face to face of the fabric and together with the weft cover the stuffer threads, providing a fabric which can be stiffened by dispersion of the soluble adhesive substance by 5 action of a solvent.

2. A woven textile fabric consisting of a two-weft plane fabric in which the wefts of each plane are separated from those of the other by a stuffer warp comprising an organically soluble adhesive 10 substance, the warp threads of which fabric pass from face to face of the fabric and together with the weft cover the stuffer warp, providing a fabric which can be stiffened by dispersion of the soluble adhesive substance by action of a solvent. 15

3. A woven textile fabric consisting of a two-weft plane fabric in which the wefts of each plane are separated from those of the other by a stuffer weft comprising an organically soluble adhesive substance, the warp threads of which fabric pass 20 from face to face of the fabric and together with the weft cover the stuffer weft, providing a fabric which can be stiffened by dispersion of the soluble adhesive substance by action of a solvent. 25

FRITZ HANFF.  
JULIUS REIMANN.